



US006939000B2

(12) **United States Patent**  
Pan et al.

(10) **Patent No.:** **US 6,939,000 B2**  
(45) **Date of Patent:** **Sep. 6, 2005**

(54) **PHASE CHANGE INK IMAGING  
COMPONENT WITH POLYMER HYBRID  
LAYER**

(75) Inventors: **David H. Pan**, Rochester, NY (US);  
**Santokh S. Badesha**, Pittsford, NY (US);  
**Xiaoying Yuan**, Fairport, NY (US);  
**Donald S. Stanton**, Penfield, NY (US);  
**Anthony Yeznach**, Clackamas, OR (US);  
**Trevor J. Snyder**, Newberg, OR (US)

(73) Assignee: **Xerox Corporation**, Stamford, CT (US)

(\*) Notice: Subject to any disclaimer, the term of this patent is extended or adjusted under 35 U.S.C. 154(b) by 4 days.

(21) Appl. No.: **10/177,908**

(22) Filed: **Jun. 20, 2002**

(65) **Prior Publication Data**

US 2003/0234839 A1 Dec. 25, 2003

(51) **Int. Cl.** <sup>7</sup> **B41J 2/01**

(52) **U.S. Cl.** **347/103**

(58) **Field of Search** **347/103; 492/56;  
428/36.8, 39.91, 319.3, 422, 447, 448,  
450, 906; 524/504, 551; 359/308, 318**

(56) **References Cited**

**U.S. PATENT DOCUMENTS**

|              |   |         |                     |       |         |
|--------------|---|---------|---------------------|-------|---------|
| 4,853,737 A  | * | 8/1989  | Hartley et al.      | ..... | 399/333 |
| 5,372,852 A  | * | 12/1994 | Titterington et al. | ..... | 427/256 |
| 5,736,250 A  | * | 4/1998  | Heeks et al.        | ..... | 428/447 |
| 6,009,298 A  | * | 12/1999 | Sakamaki et al.     | ..... | 399/318 |
| 6,312,792 B1 | * | 11/2001 | Okada et al.        | ..... | 428/220 |
| 6,500,367 B2 | * | 12/2002 | Naus et al.         | ..... | 264/39  |

\* cited by examiner

*Primary Examiner*—Anh T. N. Vo

(74) *Attorney, Agent, or Firm*—Annette L. Bade

(57) **ABSTRACT**

An offset printing apparatus having a coated imaging member for use with phase-change inks, has a substrate, an optional intermediate layer, and thereover an outer coating with a hybrid composition of an elastomer having a silicone material covalently bonded to a backbone of the elastomer, and an optional heating member associated with the offset printing apparatus.

**17 Claims, 2 Drawing Sheets**





FIG. 1



FIG. 2



**FIG. 3**

## 1

**PHASE CHANGE INK IMAGING  
COMPONENT WITH POLYMER HYBRID  
LAYER**

**CROSS REFERENCE TO RELATED  
APPLICATIONS**

Reference is made to the following commonly assigned, copending patent applications, including U.S. patent application Ser. No. 10/177,911, filed Jun. 20, 2002, entitled, "Phase Change Ink Imaging Component Having Elastomer Outer Layer;" U.S. patent application Ser. No. 10/177,909, filed Jun. 20, 2002, entitled, "Phase Change Ink Imaging Component with Outer Layer Having Haloelastomer with Pendant Chains;" U.S. patent application Ser. No. 10/177,780, filed Jun. 20, 2002, entitled, "Phase Change Ink Imaging Component with Thermoplastic Layer;" U.S. patent application Ser. No. 10/177,908, filed Jun. 20, 2002, entitled, "Phase Change Ink Imaging Component with Thermoset Layer," U.S. patent application Ser. No. 10/177,800, filed Jun. 20, 2002 entitled, "Phase Change Ink Imaging Component with Fluorosilicone Layer," U.S. patent application Ser. No. 10/177,906, filed Jun. 20, 2002, entitled, "Phase Change Ink Imaging Component with Latex Fluoroelastomer Layer," U.S. patent application Ser. No. 10/177,904, filed Jun. 20, 2002, entitled, "Phase Change Ink Imaging Component with Mica-Type Silicate Layer;" U.S. patent application Ser. No. 10/177,910, filed Jun. 20, 2002, entitled, "Phase Change Ink Imaging Component with Q-Resin Layer;" and U.S. patent application Ser. No. 10/177,779, filed Jun. 20, 2002, entitled, "Phase Change Ink Imaging Component with Polymer Blend Layer." The disclosures of each of these patent applications is hereby incorporated by reference in their entirety.

**BACKGROUND OF THE INVENTION**

The present invention relates generally to an imaging apparatus and layers for components thereof, and for use in offset printing or ink jet printing apparatuses. The layers herein are useful for many purposes including layers for transfer components, including transfix or transfuse components, imaging components, and like components. More specifically, the present invention relates to layers comprising polymer hybrids. The layers of the present invention may be useful in components used in combination with ink or dye materials. In embodiments, the layers can be used in combination with phase change inks such as solid inks.

Ink jet printing systems using intermediate transfer, transfix or transfuse members are well known, such as that described in U.S. Pat. No. 4,538,156. Generally, the printing or imaging member is employed in combination with a printhead. A final receiving surface or print medium is brought into contact with the imaging surface after the image has been placed thereon by the nozzles of the printhead. The image is then transferred and fixed to a final receiving surface.

More specifically, the phase-change ink imaging process begins by first applying a thin liquid, such as, for example, silicone oil, to an imaging member surface. The solid or hot melt ink is placed into a heated reservoir where it is maintained in a liquid state. This highly engineered ink is formulated to meet a number of constraints, including low viscosity at jetting temperatures, specific visco-elastic properties at component-to-media transfer temperatures, and high durability at room temperatures. Once within the printhead, the liquid ink flows through manifolds to be

## 2

ejected from microscopic orifices through use of proprietary piezoelectric transducer (PZT) printhead technology. The duration and amplitude of the electrical pulse applied to the PZT is very accurately controlled so that a repeatable and precise pressure pulse can be applied to the ink, resulting in the proper volume, velocity and trajectory of the droplet. Several rows of jets, for example four rows, can be used, each one with a different color.

The individual droplets of ink are jetted onto the liquid layer on the imaging member. The imaging member and liquid layer are held at a specified temperature such that the ink hardens to a ductile visco-elastic state.

After depositing the image, a print medium is heated by feeding it through a preheater and into a nip formed between the imaging member and a pressure member, either or both of which can also be heated. A high durometer synthetic pressure member is placed against the imaging member in order to develop a high-pressure nip. As the imaging member rotates, the heated print medium is pulled through the nip and is pressed against the deposited ink image with the help of a pressure member, thereby transferring the ink to the print medium. The pressure member compresses the print medium and ink together, spreads the ink droplets, and fuses the ink droplets to the print medium. Heat from the pre-heated print medium heats the ink in the nip, making the ink sufficiently soft and tacky to adhere to the print medium. When the print medium leaves the nip, stripper fingers or other like members, peel it from the printer member and direct it into a media exit path.

To optimize image resolution, the transferred ink drops should spread out to cover a predetermined area, but not so much that image resolution is compromised or lost. The ink drops should not melt during the transfer process. To optimize printed image durability, the ink drops should be pressed into the paper with sufficient pressure to prevent their inadvertent removal by abrasion. Finally, image transfer conditions should be such that nearly all the ink drops are transferred from the imaging member to the print medium. Therefore, it is desirable that the imaging member has the ability to transfer the image to the media sufficiently.

The imaging member is multi-functional. First, the ink jet printhead prints images on the imaging member, and thus, it is an imaging member. Second, after the images are printed on the imaging member, they can then transfix or transfuse to a final print medium. Therefore, the imaging member provides a transfix or transfuse function, in addition to an imaging function.

In order to ensure proper transfer and fusing of the ink off the imaging member to the print medium, certain nip temperature, pressure and compliance are required. Unlike laser printer imaging technology in which solid fills are produced by sheets of toner, the solid ink is placed on the imaging member one pixel at a time and the individual pixels must be spread out during the transfix process to achieve a uniform solid fill. Also, the secondary color pixels on the imaging member are physically taller than the primary color pixels because the secondary pixels are produced from two primary pixels. Therefore, compliance in the nip is required to conform around the secondary pixels and to allow the primary pixel neighbors to touch the media with enough pressure to spread and transfer. The correct amount of temperature, pressure and compliance is required to produce acceptable image quality.

Currently, the imaging member useful for solid inks or phase change inks comprises anodized aluminum. This member operates at about 57° C. to about 64° C. and can be

used with a heater that preheats the print media prior to entering the nip. Otherwise, the imaging member may include a heater associated therewith. The heater may be associated anywhere on the offset printing apparatus. The current aluminum-imaging member has several drawbacks. A high nip load of up to about 770 pounds is needed for transfix or transfix operations. Further, because of the high nip load, bulky mechanisms and supporting structures are needed, resulting in increased printer weight and cost. One example is that a fairly complex two-layer pressure roller is needed. In addition, the first copy out time is unacceptable because of the bulky weight. Moreover, low cohesive failure temperature is another drawback to use of an anodized aluminum drum.

Several coatings for the imaging member have been suggested. Examples are listed below.

U.S. Pat. No. 5,092,235 discloses a pressure fixing apparatus for ink jet inks having 1) outer shell of rigid, non-compliant material such as steel, or polymer such as acetal homopolymer or Nylon 6/6 and 2) an underlayer of elastomer material having a hardness of about 30 to 60, or about 50 to 60.

U.S. Pat. No. 5,195,430 discloses a pressure fixing apparatus for ink jet inks having 1) outer shell of rigid, non-compliant material such as steel, or polymer such as acetal homopolymer or Nylon 6/6 and 2) an underlayer of elastomer material having a hardness of about 30 to 60, or about 50 to 60, which can be polyurethane (VIBRATHANE, or REN:C:O-thane).

U.S. Pat. No. 5,389,958 discloses an intermediate transfer member/image receiving member having a surface of metal (aluminum, nickel, iron phosphate), elastomers (fluoroelastomers, perfluoroelastomers, silicone rubber, polybutadiene), plastics (polyphenylene sulfide), thermoplastics (polyethylene, polyamide (nylon), FEP), thermosets (metals, ceramics), and a pressure roller with elastomer surface.

U.S. Pat. No. 5,455,604 discloses a fixing mechanism and pressure wheels, wherein the pressure wheels can be comprised of a steel or plastic material such as DELRIN. Image-receiving drum 40 can be a rigid material such as aluminum or stainless steel with a thin shell mounted to the shaft, or plastic.

U.S. Pat. No. 5,502,476 teaches a pressure roller having a metallic core with elastomer coating such as silicones, urethanes, nitriles, or EPDM, and an intermediate transfer member surface of liquid, which can be water, fluorinated oils, glycol, surfactants, mineral oil, silicone oil, functional oils such as mercapto silicone oils or fluorinated silicone oils or the like, or combinations thereof.

U.S. Pat. No. 5,614,933 discloses an intermediate transfer member/image receiving member having a surface of metal (aluminum, nickel, iron phosphate), elastomers (fluoroelastomers, perfluoroelastomers, silicone rubber, polybutadiene), plastics (polyphenylene sulfide), thermoplastics (polyethylene, polyamide (nylon), FEP), thermosets (metals, ceramics), or polyphenylene sulfide loaded with PTFE, and a pressure roller with elastomer surface.

U.S. Pat. No. 5,790,160 discloses an intermediate transfer member/image receiving member having a surface of metal (aluminum, nickel, iron phosphate), elastomers (fluoroelastomers, perfluoroelastomers, silicone rubber, polybutadiene), plastics (polyphenylene sulfide), thermoplastics (polyethylene, polyamide (nylon), FEP), thermosets (metals, ceramics), or polyphenylene sulfide loaded with PTFE, and a pressure roller with elastomer surface.

U.S. Pat. No. 5,805,191 an intermediate transfer member/image receiving member having a surface of metal (aluminum, nickel, iron phosphate), elastomers (fluoroelastomers, perfluoroelastomers, silicone rubber, polybutadiene), plastics (polyphenylene sulfide), thermoplastics (polyethylene, polyamide (nylon), FEP), thermosets (metals, ceramics), or polyphenylene sulfide loaded with PTFE, and an outer liquid layer of liquid, which can be water, fluorinated oils, glycol, surfactants, mineral oil, silicone oil, functional oils such as mercapto silicone oils or fluorinated silicone oils or the like, or combinations thereof.

U.S. Pat. No. 5,808,645 discloses a transfer roller having a metallic core with elastomer covering of silicone, urethanes, nitriles, and EPDM.

U.S. Pat. No. 6,196,675 B1 discloses separate image transfer and fusing stations, wherein the fuser roller coatings can be silicones, urethanes, nitriles and EPDM.

U.S. Pat. No. 5,777,650 discloses a pressure roller having an elastomer sleeve, and an outer coating that can be metals, (aluminum, nickel, iron phosphate), elastomers (fluoroelastomers, perfluoroelastomers, silicone rubber, polybutadiene), plastics (polyphenylene sulfide with PTFE filler), thermoplastics (polyethylene, polyamide (nylon), FEP), thermosets (acetals, ceramics). Preferred is anodized aluminum.

In addition, many different types of outer coatings for transfer members, fuser members, and intermediate transfer members have been used in the electrostatographic arts using powder toner, but not with liquid inks or phase change inks. Several examples are listed herein.

U.S. Pat. No. 5,361,126 discloses an imaging apparatus including a transfer member including a heater and pressure-applying roller, wherein the transfer member includes a fabric substrate and an impurity-absorbent material as a top layer. The impurity-absorbing material can include a rubber elastomer material.

U.S. Pat. No. 5,337,129 discloses an intermediate transfer component comprising a substrate and a ceramer or grafted ceramer coating comprised of integral, interpenetrating networks of haloelastomer, silicon oxide, and optionally polyorganosiloxane.

U.S. Pat. No. 5,340,679 discloses an intermediate transfer component comprised of a substrate and thereover a coating comprised of a volume grafted elastomer, which is a substantially uniform integral interpenetrating network of a hybrid composition of a fluoroelastomer and a polyorganosiloxane.

U.S. Pat. No. 5,480,938 describes a low surface energy material comprising a volume grafted elastomer which is a substantially uniform integral interpenetrating network of a hybrid composition of a fluoroelastomer and a polyorganosiloxane, the volume graft having been formed by dehydrofluorination of fluoroelastomer by a nucleophilic dehydrofluorinating agent, followed by a hydrosilation reaction, addition of a hydrogen functionally terminated polyorganosiloxane and a hydrosilation reaction catalyst

U.S. Pat. No. 5,366,772 describes a fuser member comprising a supporting substrate, and a outer layer comprised of an integral interpenetrating hybrid polymeric network comprised of a haloelastomer, a coupling agent, a functional polyorganosiloxane and a crosslinking agent.

U.S. Pat. No. 5,456,987 discloses an intermediate transfer component comprising a substrate and a titamer or grafted titamer coating comprised of integral, interpenetrating networks of haloelastomer, titanium dioxide, and optionally polyorganosiloxane.

U.S. Pat. No. 5,848,327 discloses an electrode member positioned near the donor member used in hybrid scavengerless development, wherein the electrode members have a composite haloelastomer coating.

U.S. Pat. No. 5,576,818 discloses an intermediate toner transfer component including: (a) an electrically conductive substrate; (b) a conformable and electrically resistive layer comprised of a first polymeric material; and (c) a toner release layer comprised of a second polymeric material selected from the group consisting of a fluorosilicone and a substantially uniform integral interpenetrating network of a hybrid composition of a fluoroelastomer and a polyorganosiloxane, wherein the resistive layer is disposed between the substrate and the release layer.

U.S. Pat. No. 6,035,780 discloses a process for forming a layer on a component of an electrostatographic apparatus, including mixing a first fluoroelastomer and a polymeric siloxane containing free radical reactive functional groups, and forming a second mixture of the resulting product with a mixture of a second fluoroelastomer and a second polysiloxane compound.

U.S. Pat. No. 5,537,194 discloses an intermediate toner transfer member comprising: (a) a substrate; and (b) an outer layer comprised of a haloelastomer having pendant hydrocarbon chains covalently bonded to the backbone of the haloelastomer.

U.S. Pat. No. 5,753,307 discloses fluoroelastomer surfaces and a method for providing a fluoroelastomer surface on a supporting substrate which includes dissolving a fluoroelastomer; adding a dehydrofluorinating agent; adding an amino silane to form a resulting homogeneous fluoroelastomer solution; and subsequently providing at least one layer of the homogeneous fluoroelastomer solution to the supporting substrate.

U.S. Pat. No. 5,840,796 describes polymer nanocomposites including a mica-type layered silicate and a fluoroelastomer, wherein the nanocomposite has a structure selected from the group consisting of an exfoliated structure and an intercalated structure.

U.S. Pat. No. 5,846,643 describes a fuser member for use in an electrostatographic printing machine, wherein the fuser member has at least one layer of an elastomer composition comprising a silicone elastomer and a mica-type layered silicate, the silicone elastomer and mica-type layered silicate form a delaminated nanocomposite with silicone elastomer inserted among the delaminated layers of the mica-type layered silicate.

U.S. Pat. No. 5,933,695 discloses a rapid wake up fuser member comprising a substrate, a heat transmissive layer provided on the substrate and having a silicone material and a Q-resin, and a toner release layer comprising a polymer and provided on the heat transmissive layer.

U.S. Pat. No. 4,853,737 discloses rollers having an outer layer comprising a cured fluoroelastomer containing pendant polydiorganosiloxane units that are covalently bonded to the backbone of the fluoroelastomer.

It is desired to provide a multi-functional imaging member for use with phase change ink printing machines, which has the ability to receive an image, and either transfer, or transfer and fuse the image to a print medium. It is desired that the imaging member when having heat associated therewith, be thermally stable for conduction for fusing or fixing. It is further desired that the imaging member have a relatively low nip load, in order to decrease the weight and cost of the printing machine, and in order to provide an acceptable first copy out time.

## SUMMARY OF THE INVENTION

The present invention provides, in embodiments: an offset printing apparatus for transferring a phase change ink onto a print medium comprising: a) a phase change ink component for applying a phase change ink in a phase change ink image; b) an imaging member for accepting the phase change ink image from the phase change ink component, and transferring the phase change ink image from the imaging member to the print medium, the imaging member comprising: i) an imaging substrate, and thereover ii) an outer coating comprising a hybrid composition of an elastomer having a silicone material covalently bonded to a backbone of the elastomer.

The present invention further provides, in embodiments: an offset printing apparatus for printing a phase change ink onto a print medium comprising: a) a phase change ink component for applying a phase change ink in a phase change ink image; b) an imaging member for accepting the phase change ink image from the phase change ink component, and transferring the phase change ink image from the imaging member to the print medium and for fixing the phase change ink image to the print medium, the imaging member comprising in order: i) an imaging substrate, ii) an intermediate layer, and iii) an outer coating comprising a hybrid composition of an elastomer having a silicone material covalently bonded to a backbone of the elastomer; and c) a heating member associated with the offset printing apparatus.

In addition, the present invention provides, in embodiments: an offset printing apparatus comprising a phase change ink component containing a phase change ink; an imaging member comprising a substrate, and thereover an outer coating comprising a hybrid composition of an elastomer having a silicone material covalently bonded to a backbone of the elastomer; and a heating member associated with the offset printing apparatus, wherein the phase change ink component dispenses the phase change ink onto the imaging member, and wherein the phase change ink is solid at room temperature.

## BRIEF DESCRIPTION OF THE DRAWINGS

The above embodiments of the present invention will become apparent as the following description proceeds upon reference to the drawings, which include the following figures:

FIG. 1 is an illustration of an embodiment of the invention, and includes a transfer printing apparatus using an imaging member in the form of a drum.

FIG. 2 is an enlarged view of an embodiment of a printing drum having a substrate and an outer polymer hybrid layer thereon.

FIG. 3 is an enlarged view of an embodiment of a printing drum having a substrate, an optional intermediate layer, and an outer polymer hybrid layer thereon.

## DETAILED DESCRIPTION OF THE INVENTION

The present invention is directed to an offset printing apparatus useful with phase-change inks such as solid inks, and comprising a coated imaging member capable of accepting, transferring and in some embodiments, fixing an ink image to a print medium. The imaging member can be a roller such as a drum, or a film component such as a film, sheet, belt or the like. In embodiments, the imaging member comprises a substrate and an outer layer comprising a

polymer hybrid. In an alternative embodiment, the imaging member comprises a substrate, an optional intermediate layer, and outer layer comprising a polymer hybrid. The substrate, intermediate layer, and/or outer layer can further comprise fillers dispersed or contained therein.

The polymer hybrid coating, in embodiments, provides a reduction in transfix load from 770 pounds down to about 100 to about 300 pounds. Also, the polymer hybrid coating, in embodiments, provides a high temperature release capability while maintaining 25 ips transfix speed, and print quality of phase change inks. The polymer hybrid coating also helps to increase the temperature of the imaging member, in embodiments wherein the imaging member has heat associated therewith. The temperature can be increased from about 57° C. to about 80° C. to enable high temperature release capability. In addition, the polymer hybrid outer layer, in embodiments, helps eliminate or drastically reduce the requirement for paper preheating. Moreover, the polymer hybrid layer, in embodiments, is a compliant surface on the imaging member that reduces or eliminates the need for a complex and expensive two-layer imaging member.

The details of embodiments of phase-change ink printing processes are described in the patents referred to above, such as U.S. Pat. Nos. 5,502,476; 5,389,958; and 6,196,675 B1, the disclosures of each of which are hereby incorporated by reference in their entirety. An example of one embodiment of a phase-change ink printing process is set forth below.

Referring to FIG. 1, offset printing apparatus 1 is demonstrated to show transfer of an ink image from the imaging member to a final printing medium or receiving substrate. As the imaging member 3 turns in the direction of arrow 5, a liquid surface 2 is deposited on imaging member 3. The imaging member 3 is depicted in this embodiment as a drum member. However, it should be understood that other embodiments can be used, such as a belt member, film member, sheet member, or the like. The liquid layer 2 is deposited by an applicator 4 that may be positioned at any place, as long as the applicator 4 has the ability to make contact and apply liquid surface 2 to imaging member 3.

The ink used in the printing process can be a phase change ink, such as, for example, a solid ink. The term "phase change ink" means that the ink can change phases, such as a solid ink becoming liquid ink or changing from solid into a more malleable state. Specifically, in embodiments, the ink can be in solid form initially, and then can be changed to a molten state by the application of heat energy. The solid ink may be solid at room temperature, or at about 25° C. The solid ink may possess the ability to melt at relatively high temperatures above from about 85° C. to about 150° C. The ink is melted at a high temperature and then the melted ink 6 is ejected from printhead 7 onto the liquid layer 2 of imaging member 3. The ink is then cooled to an intermediate temperature of from about 20° C. to about 80° C., or about 72° C., and solidifies into a malleable state in which it can then be transferred onto a final receiving substrate 8 or print medium 8.

The ink has a viscosity of from about 5 to about 30 centipoise, or from about 8 to about 20 centipoise, or from about 10 to about 15 centipoise at about 140° C. The surface tension of suitable inks is from about 23 to about 50 dynes/cm. Examples of a suitable inks for use herein include those described in U.S. Pat. Nos. 4,889,560; 5,919,839; 6,174,937; and 6,309,453, the disclosure each of which are hereby incorporated by reference in their entirety.

Some of the liquid layer 2 is transferred to the print medium 8 along with the ink. A typical thickness of trans-

ferred liquid is about 100 angstroms to about 100 nanometer, or from about 0.1 to about 200 milligrams, or from about 0.5 to about 50 milligrams, or from about 1 to about 10 milligrams per print medium.

5 Suitable liquids that may be used as the print liquid surface 2 include water, fluorinated oils, glycol, surfactants, mineral oil, silicone oil, functional oils, and the like, and mixtures thereof. Functional liquids include silicone oils or polydimethylsiloxane oils having mercapto, fluoro, hydride, 10 hydroxy, and the like functionality.

Feed guide(s) 10 and 13 help to feed the print medium 8, such as paper, transparency or the like, into the nip 9 formed between the pressure member 11 (shown as a roller), and imaging member 3. It should be understood that the pressure member can be in the form of a belt, film, sheet, or other form. In embodiments, the print medium 8 is heated prior to entering the nip 9 by heated feed guide 13. When the print medium 8 is passed between the printing medium 3 and the pressure member 11, the melted ink 6 now in a malleable state is transferred from the imaging member 3 onto the print medium 8 in image configuration. The final ink image 12 is spread, flattened, adhered, and fused or fixed to the final print medium 8 as the print medium moves between nip 9. Alternatively, there may be an additional or alternative heater or heaters (not shown) positioned in association with offset printing apparatus 1. In another embodiment, there may be a separate optional fusing station located upstream or downstream of the feed guides.

The pressure exerted at the nip 9 is from about 10 to about 30,000 psi, or about 500 psi, or from about 200 to about 500 psi. This is approximately twice the ink yield strength of about 250 psi at 50° C. In embodiments, higher temperatures, such as from about 72 to about 75° C. can be used, and at the higher temperatures, the ink is softer. Once the ink is transferred to the final print medium 8, it is cooled to an ambient temperature of from about 20° C. to about 25° C.

40 Stripper fingers (not shown) may be used to assist in removing the print medium 8 having the ink image 12 formed thereon to a final receiving tray (also not shown).

FIG. 2 demonstrates an embodiment of the invention, wherein imaging member 3 comprises substrate 15, having thereover outer coating 16.

45 FIG. 3 depicts another embodiment of the invention. FIG. 3 depicts a three-layer configuration comprising a substrate 15, intermediate layer 17 positioned on the substrate 15, and outer layer 16 positioned on the intermediate layer 17. In embodiments, the outer release layer 16 comprises a polymer hybrid. In embodiments, an outer liquid layer 2 (as described above) may be present on the outer layer 16.

In embodiments, the hybrid comprises an elastomer, such as a haloelastomer. Examples of elastomers comprising halogen monomers include chloroelastomers, fluoroelastomers and the like. Examples of fluoroelastomers include ethylenically unsaturated fluoroelastomers, and fluoroelastomers comprising copolymers and terpolymers of vinylidene fluoride, hexafluoropropylene and tetrafluoroethylene, which are known commercially under various designations as VITON A®, VITON B®, VITON E®, VITON F®, VITON E60C®, VITON E45®, VITON E430®, VITON B 910®, VITON GH®, VITON B50®, VITON E45®, and VITON GF®. The VITON® designation is a Trademark of E. I. DuPont de Nemours, Inc. Three known fluoroelastomers are (1) a class of copolymers of vinylidene fluoride, hexafluoropropylene and tetrafluoroethylene, known commercially as VITON A®, (2)

a class of terpolymers of vinylidenefluoride, hexafluoropropylene and tetrafluoroethylene known commercially as VITON B®, and (3) a class of tetrapolymers of vinylidenefluoride, hexafluoropropylene, tetrafluoroethylene and a cure site monomer, for example, VITON® GF, VITON A®, and VITON B®.

In another embodiment, the fluoroelastomer is a tetrapolymer having a relatively low quantity of vinylidenefluoride. An example is VITON GF®, available from E. I. DuPont de Nemours, Inc. The VITON GF® has 35 weight percent of vinylidenefluoride, 34 weight percent of hexafluoropropylene and 29 weight percent of tetrafluoroethylene with 2 weight percent cure site monomer. The cure site monomer can be those available from DuPont such as 4-bromoperfluorobutene-1,1,1-dihydro-4-bromoperfluorobutene-1, 3-bromoperfluoropropene-1,1,1-dihydro-3-bromoperfluoropropene-1, or any other suitable, known, commercially available cure site monomer.

Other fluoroelastomer that may be used include AFLAS®, FLUOREL® I, FLUOREL® II, TECNOFLON® and the like commercially available elastomers.

In embodiments, the silicone material can be a poly(imide-organosiloxane), poly(urethane-organosiloxane) block copolymer, both having functional groups such as those functional groups defined as "X" in Formula I below, or "A" in Formula II below. In embodiments, the silicone material is a polyorganosiloxane. Any suitable polyorganosiloxane can be used. Examples include monofunctional, difunctional, and multifunctional polyorganosiloxanes.

Examples of suitable organosiloxanes include those having functional groups such as amines, phenols and thiols, which help provide covalent bonding with the backbone of the elastomer. Examples of such oligomers include those having the Formula I:



wherein R can be an alkyl from about 1 to about 24 carbons, or an alkenyl of from about 2 to about 24 carbons, or a substituted or unsubstituted aryl or heterocyclic of from about 4 to about 24 carbons such as a phenyl group or the like; or a haloalkyl such as fluoropropyl, fluorobutyl or the like; R' is an alkylene such as methylene, ethylene or isopropylene, or arylene such as phenylene; each X can be the same or different and can be a functional or nonfunctional group having an active hydrogen such as —OH, —NH<sub>2</sub>, —NR'H, —SH, —NHCO<sub>2</sub>, wherein R' is hydrogen or an alkyl having from about 1 to about 12 carbons, or from about 1 to about 6 carbons, and X can also be an end group such as a hydrogen, or an alkyl of from about 1 to about 12 carbons, or from about 1 to about 6 carbons, such as methyl, ethyl propyl, and wherein at least one of the X groups is a functional group; and wherein n, m, and o are positive integers, each n, m and o being of from about 1 to about 100, or from about 1 to about 50, or from about 1 to about 25. The average molecular weight of the organosiloxane is from about 1,000 to about 10,000, or from about 2,000 to about 14,000.

Other examples of suitable polyorganosiloxanes have the following Formula II:



where R is an alkyl from about 1 to about 24 carbons, or an alkenyl of from about 2 to about 24 carbons, or a substituted or unsubstituted aryl or heterocyclic of from about 4 to about 24 carbons; each A can be the same or different and can be an aryl or heterocyclic of from about 6 to about 24 carbons, a substituted or unsubstituted alkene of from about 2 to about 8 carbons, such as a vinyl group, a substituted or unsubstituted alkyne of from about 2 to about 8 carbons, or a substituted or unsubstituted alkoxy group having from about 2 to about 8 carbons, an amino group, or an alkyl amino group wherein the alkyl group is methyl, ethyl, propyl, butyl, pentyl and the like, and A can also be an end group such as hydrogen, alkyl of from about 1 to about 10, or from about 1 to about 6 carbons, such as methyl, ethyl, propyl, butyl, pentyl and the like, wherein at least one A groups is a functional group; and n is from about 2 to about 400, or from about 10 to about 200, in embodiments.

In embodiments, R in Formula II is an alkyl, alkenyl, aryl or heterocyclic, wherein the alkyl has from about 1 to about 24 carbons, or from about 1 to about 12 carbons; the alkenyl has from about 2 to about 24 carbons, or from about 2 to about 12 carbons; and the aryl or heterocyclic has from about 4 to about 24 carbon atoms, or from about 6 to about 18 carbons. R may be a substituted aryl or heterocyclic group, wherein the aryl or heterocyclic may be substituted with an amino, hydroxy, mercapto or substituted with an alkyl having for example from about 1 to about 24 carbons or from 1 to about 12 carbons, or substituted with an alkenyl having for example from about 2 to about 24 carbons or from about 2 to about 12 carbons. In an embodiment, R is independently selected from methyl, ethyl, and phenyl. The functional group A can be an alkene or alkyne group having from about 2 to about 8 carbon atoms, or from about 2 to about 4 carbons, optionally substituted with an alkyl having for example from about 1 to about 12 carbons, or from about 1 to about 12 carbons, or an aryl or heterocyclic group having for example from about 6 to about 24 carbons, or from about 6 to about 18 carbons. Functional group A can also be mono-, di-, or trialkoxysilane having from about 1 to about 10, or from about 1 to about 6 carbons in each alkoxy group, hydroxy, or halogen. Examples of alkoxy groups include methoxy, ethoxy, and the like. Examples of halogens include chlorine, bromine and fluorine. "A" in Formula II may also be an alkyne of from about 2 to about 8 carbons, optionally substituted with an alkyl of from about 1 to about 24 carbons or aryl or heterocyclic of from about 6 to about 24 carbons. "A" can also be an amine group or an alkyl amino group such as aminomethyl, aminoethyl, aminopropyl, aminoethyl aminopropyl, aminobutyl, and the like. The group n is from about 2 to about 400, and in embodiments from about 2 to about 350, or from about 5 to about 100. Furthermore, in an embodiment, n is from about 60 to about 80 to provide a sufficient number of reactive groups to graft onto the fluoroelastomer. In the above Formula II, typical R groups include methyl, ethyl, propyl, octyl, vinyl, allylic crotyl, phenyl, naphthyl and phenanthryl, and typical substituted aryl groups are substituted in the ortho, meta and para positions with lower alkyl groups having from about 1 to about 15 carbon atoms. Typical alkene and alkenyl functional groups include vinyl,

## 11

acrylic, crotonic and acetetyl which may typically be substituted with methyl, propyl, butyl, benzyl, tolyl groups, and the like.

In embodiments, the polyorganosiloxane is an amino-functional siloxane such as aminopropyl-terminated polydimethylsiloxanes, such as DMSA-11, 12, 15 and 21, and aminopropyl methylsiloxane-dimethylsiloxane copolymers, such as ASM-132, 152, and 162, or other polyorganosiloxanes such as ASM-233, 242 and ATM 1112 or 1322, all from Gelest, Inc.

In embodiments, the polyorganosiloxane can be functional poly(dimethylsiloxanes) and silicone resins with auxiliaries such as RT601A Elastosil, or hydrogen-functional dimethylsiloxanes such as RT601B Elastosils from Wacker.

In embodiments, the polyorganosiloxane can be difunctional polydiorganosiloxanes such as  $\alpha$ ,  $\omega$ -difunctional polydiorganosiloxanes, such as bis(aminopropyl) terminated polydimethylsiloxanes.

The hybrid composition comprises an elastomer having a silicone material covalently bonded to the backbone of the elastomer. In embodiments, the silicone material is covalently bonded to the backbone of a non-cured elastomer. In embodiments, a polydiorganosiloxane segment is covalently bonded to the backbone of a non-cured fluoroelastomer. Such segments are bonded to the backbone of the cured elastomer such as a fluoroelastomer, as opposed to being an integral part of that backbone as would be the case in a random or block copolymer comprising fluorocarbon moieties. Accordingly, these silicone materials, or in embodiments, polydiorganosiloxane segments, are frequently referred to herein as being pendant polydiorganosiloxane segments. The required silicone or diorganosiloxane segments can be conveniently appended to the backbone of the cured fluoroelastomer during curing of the elastomer or fluoroelastomer base polymer, by simply adding to the composition to be cured, a silicone or polydiorganosiloxane oligomer containing appropriate functional groups such as phenoxy or amino groups. At least one of these functional groups must be present on a silicone or polydiorganosiloxane chain in the oligomer to form the covalent bond the elastomer or fluoroelastomer backbone. Such groups react with the elastomer or fluoroelastomer base polymer as a result of dehydrofluorination of the base polymer, which takes place during curing.

The elastomer base polymers can be cured using a basic nucleophile cure system of the type described in U.S. Pat. Nos. 4,257,699, 4,264,181, and 4,272,179. Such a cure system generally employs a bifunctional agent such as a bisphenol or a diamine carbamate to generate a covalently crosslinked polymer network formed by the application of heat following basic dehydrofluorination of the polymer. The basic dehydrofluorination reaction requires the presence

## 12

in the formulation being cured of a basic metal oxide such as magnesium oxide, calcium oxide or lead oxide. The basic metal oxide reacts with acidic by-products that are believed to include hydrogen fluoride and/or derivatives thereof, that are generated during curing of the fluoroelastomer. The incorporation of a silicone or polydiorganosiloxane oligomer containing appropriate reactive groups with the essential ingredients of a basic nucleophilic addition curing system results in covalently bonding pendant polydiorganosiloxane segments to the backbone of the fluoroelastomer base polymer while it is being cured. Depending upon the number of the reactive groups on the polydiorganosiloxane oligomer, the pendant segments can form branches on the fluorocarbon backbone of the fluoroelastomer base polymer and/or enter into the crosslink network of the cured fluoroelastomer. The primary reactions involved in the basic nucleophile curing system described in the aforementioned three U.S. Patents are also disclosed and discussed in various journals and articles including a paper entitled "Viton Fluoroelastomer Crosslinking by Bisphenols" written by W. W. Schmiegel and presented at the South German Meeting of the Deutsche Dautshuk Und Gummi Gesellschaft, Apr. 28-29, 1977. One example of the nucleophilic addition cure system is the bisphenol crosslinking agent with organophosphonium salt accelerator. Another example of the nucleophilic addition cure system is crosslinking with a diamine carbamate type curing agent commonly known as DIAK 1. The following scheme demonstrates three separate reactions represents the curing of copoly(vinylidene fluoride-hexafluoropropylene) with diamine carbamate as the curing or crosslinking agent: where step 1 is the loss of HF in the presence of a base; step 2 is the insertion of the diamine carbamate agent; and step 3 is post cure in the presence of heat. Examples of diamine carbamate cure systems are hexamethylenediamine carbamate known commercially as DIAK No. 1 and N,N'-dicinnamylidene-1, 6-hexanediamine known commercially as DIAK No. 3 (DIAK is a trademark of E. I. DuPont & Co.).

Most hybrid compositions do not require any additional curatives. For instance, multi-amino functional polyorganosiloxane (functionality greater or equal to 2 per segment) can be used to actually cure the fluoroelastomer by dehydrofluorination, followed by nucleophilic addition of the amino group to the double bonds.

Other curing methods use amino silanes as curatives, such as AO 700 (N-(2-aminoethyl)-3-aminopropyl trimethoxysilane), and are described in commonly-assigned U.S. patents, such as U.S. Pat. Nos. 5,753,307; 5,750,204; 5,695,878 and 5,700,568, the disclosure of each of these patents is hereby incorporated by reference in their entirety.

An example of potential synthesis can be demonstrated in the following scheme, wherein n is defined as in Formula II:



-continued



The polymer hybrid is present in the imaging outer layer in an amount of from about 95 to about 35 percent, or from about 90 to about 50 percent, or from about 80 to about 70 percent by weight of total solids. Total solids as used herein refers to the total amount by weight of hybrid, filler, and any additional additives, fillers or like solid materials.

The hardness of the outer polymer hybrid layer is typically from about 10 to about 95 Shore A, or from about 60 to about 95 Shore A.

In embodiments, the thickness of the outer polymer hybrid layer imaging layer is from about 0.5 to about 20 mils, or from about 0.5 to about 6 mils, or from about 1 to about 4 mils.

The substrate, optional intermediate layer, and/or outer layer, in embodiments, may comprise fillers dispersed therein. These fillers can have the ability to increase the material hardness or modulus into the desired range.

Examples of fillers include fillers such as metals, metal oxides, doped metal oxides, carbon blacks, ceramics, polymers, and the like, and mixtures thereof. Examples of suitable metal oxide fillers include titanium dioxide, tin (II) oxide, aluminum oxide, indium-tin oxide, magnesium oxide, copper oxide, iron oxide, silica or silicon oxide, and the like, and mixtures thereof. Examples of carbon fillers include carbon black (such as N-990 thermal black, N330 and N110 carbon blacks, and the like), graphite, fluorinated carbon (such as ACCUFLUOR® or CARBOFLUOR®), and the like, and mixtures thereof. Examples of ceramics include silicates such as zirconium silicate, boron nitride, aluminum nitride, and the like, and mixtures thereof. Examples of polymer fillers include polytetrafluoroethylene powder, polypyrrole, polyacrylonitrile (for example, pyrolyzed polyacrylonitrile), polyaniline, polythiophenes, and the like, and mixtures thereof. In embodiments, the filler is carbon black. In embodiments, the carbon black filler is present in the polymer blend outer layer. The optional filler is present in the substrate, optional intermediate layer, and/or outer layer in an amount of from about 0 to about 50 percent, or from about 1 to about 30 percent by weight of total solids in the layer. Total solids by weight, as used herein, refers to the total amount by weight of hybrid polymer, fillers, additives, and any other solids.

The imaging substrate can comprise any material having suitable strength for use as an imaging member substrate. Examples of suitable materials for the substrate include metals, fiberglass composites, rubbers, and fabrics. Examples of metals include steel, aluminum, nickel, and their alloys, and like metals, and alloys of like metals. The thickness of the substrate can be set appropriate to the type of imaging member employed. In embodiments wherein the substrate is a belt, film, sheet or the like, the thickness can be from about 0.5 to about 500 mils, or from about 1 to about 250 mils. In embodiments wherein the substrate is in the form of a drum, the thickness can be from about  $1/32$  to about 1 inch, or from about  $1/16$  to about  $5/8$  inch.

Examples of suitable imaging substrates include a sheet, a film, a web, a foil, a strip, a coil, a cylinder, a drum, an

endless strip, a circular disc, a belt including an endless belt, an endless seamed flexible belt, an endless seamless flexible belt, an endless belt having a puzzle cut seam, a weldable seam, and the like.

In an optional embodiment, an intermediate layer may be positioned between the imaging substrate and the outer layer. Materials suitable for use in the intermediate layer include silicone materials, elastomers such as fluoroelastomers, fluorosilicones, ethylene propylene diene rubbers, and the like, and mixtures thereof. In embodiments, the intermediate layer is conformable and is of a thickness of from about 2 to about 60 mils, or from about 4 to about 25 mils.

Specific embodiments of the invention will now be described in detail. These examples are intended to be illustrative, and the invention is not limited to the materials, conditions, or process parameters set forth in these embodiments. All parts are percentages by weight of total solids as defined above unless otherwise indicated.

## EXAMPLES

### Example 1

#### Preparation of Fluoroelastomer and Silicone Hybrid Imaging Member

An aluminum substrate imaging member having the dimensions of about 10 inches long, about 4 inches in diameter, and about 0.25 inches thick, was first sanded with 400 grit sand paper, cleaned with solvent, and primed with 40 AO700, an N-(2-aminoethyl)-3-aminopropyl trimethoxysilane from United Chemical Technologies, Inc. of Bristol, Pa.

A polymer hybrid outer coating was prepared by mixing 30.75 grams of VITON® GF from DuPont Dow Elastomers, 2.1 grams of DMSA-11  $\alpha$ ,  $\omega$ -aminopropyl terminated siloxane from Gelest, 77.0 grams of methyl ethyl ketone (MEK), 611.0 grams of methyl isobutyl ketone (MiBK), and 80.0 grams of N-methyl pyrrolidinone (NMP). The mixture was then mixed with a paint-shaker until a uniform solution was obtained. No curative was used for this polymer hybrid composition since DMSA-11 can cross-link VITON® GF.

The polymer hybrid solution was coated onto the above primed aluminum drum substrate using a spray coater. The following spray conditions were used:

Binks model 21 air atomization spray gun

Fluid Nozzle: 63 B

Air Nozzle: 63 PB

Fluid Pressure: 2.25 lbs.

Air Flow: 300 cf/min.

Needle Setting: 1.0 turns open

Fan Angle: 0.75 turns open.

After the coating was air dried overnight, the coated imaging member was then post-cured. The curing was accomplished by heating the outer coating on the imaging member at 50 and 75° C. for about 1 hour, then at 95° C., 146° C., 176° C. and 205° C. each for about 2 hours, and then at 232° C. for about 6 hours.

## 15

## Example 2

## Preparation of Cured Fluoroelastomer Hybrid with Carbon Filler Coating for Imaging Member

The VITON® hybrid can be cured or chemically crosslinked to an elastomer by use of curative material VC-50, a Bisphenol AF (0-90%) benzyltriphenyl phosphonium Bisphenol AF Salt (10-100%) from DuPont Dow Elastomers. Alternatively, the curative AO700, an N-(2-aminoethyl)-3-aminopropyl trimethoxysilane from United Chemical Technologies, Inc. of Bristol, Pa. can be used. The VC-50 is used at 5 percent by weight of the VITON®, or AO700 is used at about 5 percent by weight of the VITON®. However, the AO700 is not used in this example.

A carbon black filled VITON® B50 compound was prepared by mixing 400 grams of VITON® B50 from DuPont Dow Elastomers, 60 grams of super-abrasion N110 carbon black filler from R. T. Vanderbilt Company, 8 grams of Elastomag 170S magnesium oxide, and 4 grams of calcium hydroxide from J. T. Baker in a two roll mill.

About 80 grams of the above compound was then added to 320 grams of MiBK and well mixed in a paint-shaker for about 16 hours until the dispersion was uniform and smooth. The dispersion contained 20% solids by the total weight.

A VC-50 MEK solution was prepared by mixing 3.39 grams of VC-50 and 10.17 grams of MEK solvent. The VC-50 solution and 10.17 grams of DMSA-15  $\alpha,\omega$ -aminopropyl terminated siloxane from Gelest were then added the above 400 grams of the coating dispersion. The mixture was rolled for 15 minutes before delivery to the coating line.

The resulting N110 carbon filled fluoroelastomer silicone hybrid coating composition was coated onto an imaging member using a flow coater consisting of a mechanical drive to rotate the drum and a solution dispenser and metering blade to level the fluid coating. The drum was rotated at 100 RPM and the solution flow rates was about 22.95 gms/minute to obtain a 20-micrometer thick coating on the drum with curing. The procedure was repeated with the same or different flow rate to achieve a thicker coating of the VITON® B50 hybrid composition on the surface of the drum.

The polymer hybrid with N110 carbon filler, after curatives were added and coating was coated onto an imaging member, was step heat cured as follows: 50° C. and 75° C. for about 1 hour, then at 95° C., 146° C., 176° C. and 205° C. each for about 2 hours, and then at 232° C. for about 6 hours.

While the invention has been described in detail with reference to specific and preferred embodiments, it will be appreciated that various modifications and variations will be apparent to the artisan. All such modifications and embodiments as may readily occur to one skilled in the art are intended to be within the scope of the appended claims.

We claim:

1. An offset printing apparatus for transferring a phase change ink onto a print medium comprising: 55
  - a phase change ink component for applying a phase change ink in a phase change ink image;
  - an imaging member for accepting the phase change ink image from the phase change ink component, and transferring the phase change ink image from the imaging member to the print medium, the imaging member comprising:
    - i) an imaging drum substrate, and thereover
    - ii) an outer coating comprising a hybrid composition of 65 an elastomer having a silicone material covalently bonded to a backbone of the elastomer.

## 16

2. The offset printing apparatus of claim 1, wherein said elastomer is a haloelastomer.

3. The offset printing apparatus of claim 2, wherein the haloelastomer is a fluoroelastomer.

4. The offset printing apparatus of claim 3, wherein said fluoroelastomer is selected from the group consisting of a) copolymers of vinylidenefluoride, hexafluoropropylene, and tetrafluoroethylene, b) terpolymers of vinylidenefluoride, hexafluoropropylene and tetrafluoroethylene, and c) tetrapolymers of vinylidenefluoride, hexafluoropropylene, tetrafluoroethylene, and a cure site monomer.

5. The offset printing apparatus of claim 4, wherein the fluoroelastomer comprises of 35 weight percent of vinylidenefluoride, 34 weight percent of hexafluoropropylene, 29 weight percent of tetrafluoroethylene, and 2 weight percent cure site monomer.

6. The offset printing apparatus of claim 1, wherein the silicone material is a polyorganosiloxane.

7. The offset printing apparatus of claim 6, wherein said polyorganosiloxane is mono-, di- or multi-functional.

8. The offset printing apparatus of claim 7, wherein the polyorganosiloxane monomer comprises functionality selected from the group consisting of vinyl, alkoxy and amino functionality.

9. The offset printing apparatus of claim 8, wherein said polyorganosiloxane is an  $\alpha,\omega$ -difunctional polydiorganosiloxane.

10. The offset printing apparatus of claim 9, wherein said polyorganosiloxane is a bis(aminopropyl) terminated polydimethylsiloxane.

11. The offset printing apparatus of claim 1, wherein said elastomer is a fluoroelastomer and said silicone material is a polyorganosiloxane.

12. The offset printing apparatus of claim 11, wherein said fluoroelastomer is selected from the group consisting of a) copolymers of vinylidenefluoride, hexafluoropropylene, and tetrafluoroethylene, b) terpolymers of vinylidenefluoride, hexafluoropropylene and tetrafluoroethylene, and c) tetrapolymers of vinylidenefluoride, hexafluoropropylene, tetrafluoroethylene, and a cure site monomer; and wherein the polyorganosiloxane is a bis(aminopropyl) terminated polydimethylsiloxane.

13. The offset printing apparatus of claim 1, wherein the outer coating further comprises a filler.

14. The offset printing apparatus of claim 13, wherein the filler is selected from the group consisting of carbon blacks, metal oxides, polymers, and mixtures thereof.

15. The offset printing apparatus of claim 1, wherein the phase change ink is solid at about 25° C.

16. The offset printing apparatus of claim 1, wherein the phase change ink comprises a dye.

17. An offset printing apparatus comprising:
  - a phase change ink component containing a phase change ink;
  - a imaging member comprising:
    - i) a drum substrate, and thereover
    - ii) an outer coating comprising a hybrid composition of an elastomer having a silicone material covalently bonded to a backbone of the elastomer; and
  - c) a heating member associated with the offset printing apparatus, wherein the phase change ink component dispenses the phase change ink onto the imaging member, and wherein the phase change ink is solid at about 2500° C.